

## UNITED STATES PATENT OFFICE.

FRANK FRED KUHN, OF MINNEAPOLIS, MINNESOTA, ASSIGNOR TO LYNDY M. LEY,  
OF MINNEAPOLIS, MINNESOTA.

## POLISHING COMPOSITION.

No Drawing.

Application filed September 22, 1922. Serial No. 589,922.

To all whom it may concern:

Be it known that I, FRANK FRED KUHN, a citizen of the United States, residing at Minneapolis, in the county of Hennepin and State of Minnesota, have invented certain new and useful Improvements in Polishing Composition, of which the following is a specification.

This invention relates to a polishing composition, and the object is to provide a new and improved composition of ingredients, which, when properly proportioned and compounded, applied to a hard surface such as a piece of furniture or an automobile, and thoroughly rubbed in and down with a suitable cloth, will produce a hard glossy finish capable of retaining itself as such and thus adding to the looks and durability of the object.

10 The composition, when ready for use is of a liquid consistency and is composed in the main of the following ingredients: turpentine, light paraffin oil, boiled linseed oil, ammonia, vinegar and liquid ether.

15 The proportioning and mixing of the various ingredients are effected preferably about as follows: To six ounces of turpentine is added fifty-seven and one-half ounces of the paraffin oil, twenty-two ounces of the boiled linseed oil and ten ounces of a ten per cent solution of ammonia. After this mixture has stood for about ten minutes thirty-two ounces of vinegar and one-fourth ounce of the ether are added.

20 After the above mixture has stood for about fifteen minutes it is thoroughly agitated until it takes on a light creamy color, at which time it is filled into bottles or cans.

The agitation continues during the filling process so as to cause the proper proportions of each ingredient to be filled into each bottle or can, as the case may be.

When using the polish it is necessary to first shake the container well. It is then applied to the surface and rubbed down with a soft cloth in much the same manner as all other polishes are usually applied.

It is understood that the proportions of the various ingredients may be modified, as may at times be found desirable, and such changes or modifications in the invention, it is understood, may be made, provided they come within the spirit and scope of the appended claims.

Having now therefore fully disclosed my invention what I claim is:

1. A polishing composition comprising turpentine, paraffin oil and linseed oil in substantially the following amounts: turpentine, six ounces; paraffin oil, fifty-seven ounces; and linseed oil, twenty-two ounces.

2. A polishing composition comprising turpentine, paraffin oil, linseed oil and ammonia in substantially the following amounts: turpentine, six ounces; paraffin oil, fifty-seven ounces; linseed oil, twenty-two ounces; and ten ounces of a ten per cent solution of ammonia.

3. A polishing composition consisting of six ounces of turpentine, fifty-seven ounces of paraffin oil, twenty-two ounces of boiled linseed oil, ten ounces of a ten per cent solution of ammonia, thirty-two ounces of vinegar, and, one-fourth ounce of ether.

In testimony whereof I affix my signature.

FRANK FRED KUHN.